

## 1

2,927,875

## PROCESS FOR CARBURIZING AND CARBONITRIDING IRON AND STEEL

Johannes Müller, Frankfurt am Main, Germany, assignor to Deutsche Gold- und Silber-Scheideanstalt vormals Roessler, Frankfurt (Main), Germany

No Drawing. Application June 20, 1958  
Serial No. 743,467

Claims priority, application Germany June 26, 1957

8 Claims. (Cl. 148—15.5)

The present invention relates to an improved process for carburizing and carbonitriding iron and steels in cyanide and cyanate containing salt baths whereby especially increased case depths can be obtained.

It is known that iron and steel articles can be cemented, that is, carburized to a certain depth below their surface by treatment in fused salt baths containing cyanides. The salt baths which are known for this purpose contain one or more cyanides as the carbon source and substantial proportions of alkali metal and/or alkaline earth metal halides. The decrease in carbon content with increased distance from the surface of the articles and therefore also the time required for the carburization depends essentially upon the cyanide content of the salt bath, the presence or absence of accelerators or activators, such as, for example, certain alkaline earth metal halides, and particularly the carburizing temperature employed.

Baths without an activator produce a low carbon content in the edge zone but the nitrogen which is simultaneously split off from the cyanide produces a high surface hardness. However, deep case depths cannot be achieved with such baths and the cases cannot be ground off without causing the hardness to decrease strongly. On the other hand, such baths are suited for the production of very thin carburization cases at temperatures below the pearlite point, above 600° C. and preferably about 650—700° C. The cases thus obtained are very hard and in view of the low temperatures employed the distortions produced by such treatment are only very slight. It was, however, previously not possible to increase the case depth obtained sufficiently so that this technique is only seldom used.

Baths without an activator in general contain more than 40% of cyanide. Because of high cyanide losses at high temperatures such baths are only operated at temperatures below 900° C. In salt baths which contain additions which promote the liberation of carbon, the cyanide content is considerably lower and usually is about 10% and barium chloride in a quantity of about 50 to 55% is present as the main constituent of the bath. The usual working temperature of such baths is about 930° C. and the use of substantially higher temperatures which would accelerate the carburization is generally not possible, as otherwise impractically high cyanide losses are engendered.

It has also been proposed to carburize iron and steels with cyanide containing baths predominantly composed of barium salts, such as barium chloride, at bath temperatures up to 1100° C. in order to increase the depth of the carburization case.

According to the invention it was found that the carbonitriding as well as the carburizing in cyanide and cyanate containing fused salt baths can be carried out in a short time to produce substantially greater case depths than previously were known, when such salt baths in addition oxygen at least contain one of the elements selenium and tellurium.

## 2

As in general cyanide containing baths a small quantity of cyanate is automatically produced, an oxygen content in the baths is automatically provided so that it is only necessary to add at least one of the other elements, tellurium or selenium to such baths. In general, 0.05 to

5 5% of such added element or elements suffices and preferably a quantity between 0.2% and 3% is employed. According to the process of the invention the baths contain 5 to 40% KCN or equivalent amounts of e.g. 10 NaCNO, LiCNO, RbCNO and the like as well as 0.1 to 60% NaCN or equivalent amounts of e.g. KCN; LiCN, RbCN, Ca(CN)<sub>2</sub> and the like. The remainder consists essentially of carbonates and halogenides especially chlorides and fluorides of alkaline metals and 15 eventually of earth alkaline metals. Small quantities of oxides are nearly always present. Mixtures of Na/KCO<sub>3</sub> and Na/KCl are very suitable. Also good yields are obtained with fluorides. The fused salt bath temperatures employed according to the invention lie between 600 20 and 1100° C., preferably between 650° and 100° C. Expediently, temperatures between 650° and 930° C. are used.

The following examples will serve to illustrate the unexpectedly improved results obtained with the process 25 according to the invention.

### Example 1

To a bath of 47% NaCN, 35% KCNO and the remainder K/NaCO<sub>3</sub>, 0.5% sodium selenide are added. 30 Samples of nearly carbon free steel (Armco-iron with 0.05% carbon) were treated in this bath at a temperature of 700° C. for 2 hours. Thereafter the thickness of the so-called transition zones and the total thickness of the case obtained on the treated samples were determined microscopically. The total thickness was 0.14 mm. and the thickness of the transition zone was 0.04 mm.

### Example 2

40 To a bath of 5% NaCN, 15% KCNO and the remainder Na/K chloride, 0.5% sodium selenide are added. Samples of a low carbon steel (containing 0.15% carbon) were treated in this bath at a temperature of 650° C. for 2 hours. Thereafter the thickness of the so-called transition zones and the total thickness of the case obtained on the treated samples were determined microscopically. The total thickness was 0.145 mm. and the thickness of the transition zone was 0.025 mm.

### Example 3

50 To a bath of 50% NaCN, 15% KCNO and the remainder potassium carbonate, 0.7% sodium telluride are added. Samples of a low carbon steel (containing 0.15% of carbon) were treated in this bath at a temperature of 700° C. for 2 hours. Thereafter the thickness of the so-called transition zones and the total thickness of the case obtained on the treated samples were determined microscopically. The total thickness was 0.17 mm. and the thickness of the transition zone was 0.02 mm.

### Example 4

A bath of 50% sodium cyanide, 10% sodium cyanate and the remainder sodium carbonate was compared with a bath of the same composition having 1% of selenium added thereto in the form of sodium selenite. Samples of a low carbon steel (containing 0.15% of carbon) were treated in such baths at a temperature of 700° C. for 1, 2, 5 and 10 hours. Thereafter the thickness of the so-called transition zones and the total thickness of the case obtained on the treated samples were determined microscopically. The following table compares the thicknesses attained.

| Hours   | Without Se           |                  | With Se              |                  |
|---------|----------------------|------------------|----------------------|------------------|
|         | Total Thickness, mm. | Trans. Zone, mm. | Total Thickness, mm. | Trans. Zone, mm. |
| 1.....  | 0.038                | 0.005            | 0.06                 | 0.01             |
| 2.....  | 0.038                | 0.01             | 0.084                | 0.04             |
| 5.....  | 0.038                | 0.012            | 0.21                 | 0.14             |
| 10..... | 0.038                | 0.038            | 0.32                 | 0.25             |

The portion of the case not forming a part of the transition zone was essentially martensitic. It will be seen that, even only after 1 hour's treatment, the total thickness of the case was substantially greater when the selenium containing bath was employed. The thickness of the transition zone is even approximately twice that when the bath in which the selenium was omitted was employed. The ratio becomes worse with longer treating periods but is noticeably still to the detriment of the bath not containing selenium. It is particularly remarkable, however, that in selenium free baths the sum of thicknesses of the martensitic zone and the transition zone does not increase upon increase of the treating period from 1 to 10 hours, whereas in selenium containing baths the thickness increases over five fold.

Analogous results were obtained with tests carried out at higher temperatures. Also, replacement of the selenium by tellurium provides an increase of the same order in the carburizing and nitriding action of the baths.

Generally, according to the process of the invention, case hardening steels are treated.

This application is co-pending with my application Serial No. 688,712, filed October 7, 1957, now Patent No. 2,875,095.

I claim:

1. A process for carburizing and carbonitriding iron and steel which comprises treating such metals in a fused salt bath containing cyanides equivalent to 0.1-60% of NaCN as well as cyanates equivalent to 5-40% of KCNO and the remainder essentially consisting of carbonates and halides of alkali and alkaline earth metals, to which 0.05-5% of at least one element selected from

the group consisting of selenium and tellurium has been added, said salt bath being maintained at a temperature between 600° and 1100° C.

2. The process of claim 1 in which the temperature of said salt bath is maintained between 650° and 930° C.

3. The process of claim 1 in which said cyanides and cyanates are alkali metal cyanides and alkali metal cyanates.

4. The process of claim 1 in which said cyanides and cyanates are alkaline earth metal cyanides and alkaline earth metal cyanates.

5. The process of claim 1 in which said added element is selenium.

6. The process of claim 1 in which said added element is tellurium.

7. A process for carburizing and carbonitriding iron and steel which comprises treating such metals in a fused salt bath containing alkali metal cyanides equivalent to 0.1-60% of NaCN as well as alkali metal cyanates equivalent to 5-40% KCNO and the remainder essentially consisting of carbonates and halides of alkali and alkaline earth metals, to which 0.05-5% of selenium has been added, said salt bath being maintained at a temperature between 600° and 1100° C.

8. A process for carburizing and carbonitriding iron and steel which comprises treating such metals in a fused salt bath containing alkali metal cyanides equivalent to 0.1-60% of NaCN as well as alkali metal cyanates equivalent to 5-40% KCNO and the remainder essentially consisting of carbonates and halides of alkali and alkaline earth metals, to which 0.05-5% of tellurium has been added, said salt bath being maintained at a temperature between 600° and 1100° C.

35 References Cited in the file of this patent

Troup: "Materials and Methods," vol. 44, September 1956, pages 110-113 (TA 401 M5).

Johnson: "Metal Working and Heat Treatment Manual," vol. III, pages 55-64, page 55 relied upon (TS 205 J6 V3).

"Materials and Methods," vol. 25, March 1947, page 108 (TA 401 M5).